

## UNITED STATES PATENT OFFICE

RUDOLPH R. ROSENBAUM, OF CHICAGO, ILLINOIS

## LUBRICANT

No Drawing. Original application filed June 18, 1928, Serial No. 286,492. Divided and this application filed July 14, 1927. Serial No. 205,848.

My invention relates to lubricants, particularly to an improved lubricant product or base to be used in the compounding of lubricating oils such as motor oils.

5 My improved base comprises primarily petroleum oil and a metallic soap to which are added an element for preventing jelling or stringing, and miscible vegetable castor oil. When such base is added to petroleum lubricating oils the resulting compound is a very 10 efficient lubricant particularly for internal combustion engines and is especially useful for preventing the formation of hard glazed surfaces as, for example, on friction bands 15 such as are used in planetary transmissions.

In such lubricating compounds a high percentage of the metallic soap is very desirable. I preferably use a water insoluble metallic soap such as aluminum oleate, zinc oleate, aluminum stearate, or zinc stearate. I 20 have found that, ordinarily, with a petroleum natural oil of say about 200" to 300" (Saybolt) viscosity at 100° F., the maximum amount of soap which can be added without 25 causing jelling or stringing is less than 5%. If more is dissolved in the oil the whole mass will turn into a jell-like substance when cooled to atmospheric temperature. An important object of my invention is, therefore, to make it possible to use as high as 20%, 30 or more, of the soap, and I accomplish this by adding a lead soap, such as lead oleate or lead naphthenate. I have found that even a 35 very small proportion, one-half of one per cent, or less, of the lead soap will not only prevent the jell formation but will make the resulting compound of absolutely stable viscosity on standing. If miscible castor oil is added the lubricating qualities and the non-chatter properties will be greatly increased and strengthened.

To produce my improved base the petroleum oil is heated and the water insoluble metallic soap is gradually added to the oil 45 during heating to become thoroughly dissolved therein, and then during heating of this mixture the lead soap is added. Castor oil may also be added but such oil must be thoroughly and permanently miscible with 50 petroleum lubricating oils. Ordinarily com-

mercial castor oil is not so miscible but in my co-pending application Serial Number 286,492, filed June 18, 1928, now Patent No. 1,773,203, dated Aug. 19, 1930, as a division out of this application, I disclose a process 55 for producing miscible castor oil and it is such castor oil that I use in my improved base.

For example, a proportion which I have employed and found very efficient, is as follows:—

55% petroleum neutral oil of 200" to 300" viscosity (Saybolt) at 100° Fahrenheit.

20% metallic soap such as aluminum oleate.

1% lead soap such as lead oleate or lead 60 naphthenate.

24% miscible castor oil.

The petroleum oil is heated up to from 400° to 500° F. and during such heating the aluminum oleate is gradually added up to the 70 full amount to become thoroughly and uniformly dissolved in the oil. If such mixture with the 20% soap content were allowed to cool it would become a thick jell. However, if during the heating process, the lead soap is 75 added to the mixture and thoroughly dissolved therein, the resulting product will not jell or become stringy upon cooling. Not only will the small quantity of lead soap prevent the aluminum oleate from causing jelling, but the resulting compound will be of 80 absolutely stable viscosity on standing.

Such compound of petroleum oil with the 20% of water insoluble soap made possible by the addition of only 1% lead soap, will be 85 an efficient base to be added to petroleum lubricating oils to produce a highly efficient motor oil and non-chatter lubricant. By the addition of the miscible castor oil a compound will result whose lubricating and non-chatter properties are greatly increased and strengthened. In compounding the base with lubricating oil the proportion of the base ranges from 5 to 20%.

As another example, the following proportions have been used;

3500 lbs. petroleum oil—200" to 300" viscosity (Saybolt) at 100° Fahr.

850 lbs. aluminum oleate.

80 to 100 lbs. lead oleate.

100

75 to 200 lbs. miscible castor oil—depending on the strength desired.

400°—450° F.—heating temperature.

Having described my invention, I claim as

5 follows:

1. A lubricating compound comprising a mineral oil, miscible castor oil, and water insoluble metallic soap.
2. A lubricant base comprising petroleum oil, aluminum oleate, and lead soap.
- 10 3. A lubricant base comprising petroleum oil, aluminum oleate, lead oleate and miscible castor oil.
- 15 4. A lubricant base comprising about 55% petroleum oil, about 20% aluminum oleate, about 1% lead oleate, and about 24% miscible castor oil.
- 20 5. A lubricating compound comprising a mineral oil, miscible castor oil, and water insoluble metallic soaps one of which is lead soap.
6. A lubricant compound comprising petroleum oil, aluminum soap, and lead soap.
- 25 7. A lubricant compound comprising petroleum oil, aluminum oleate, lead soap, and miscible castor oil.
8. A lubricant compound comprising about 80% lubricating oil, about 20% water insoluble metallic soap other than lead soap, and
- 30 9. A lubricating compound comprising a petroleum oil, water insoluble metallic soap of the group consisting of aluminum and zinc soaps, and a lead soap.
- 35 10. A lubricant compound comprising petroleum oil, lead oleate and water insoluble metallic soap of the group consisting of aluminum and zinc soaps.
11. A lubricant compound comprising
- 40 mineral oil, lead naphthenate, and water insoluble metallic soap of the group consisting of aluminum and zinc soaps.

In witness whereof, I hereunto subscribe my name this 8th day of July, 1927.

45 RUDOLPH R. ROSENBAUM.